

## UNITED STATES PATENT OFFICE

2,186,018

METHOD OF PREVENTING RUSTING OF  
FERROUS METAL SURFACESWilliam K. Griesinger, Lansdowne, Pa., assignor  
to The Atlantic Refining Company, Philadelphia, Pa., a corporation of PennsylvaniaNo Drawing. Application November 26, 1937,  
Serial No. 175,572

1 Claim. (Cl. 91—68)

The present invention relates to a method for inhibiting or preventing the rusting of ferrous metal surfaces, and particularly iron or steel surfaces which may be subjected to conditions normally conducive to rusting. The present invention is particularly applicable to the prevention of rusting of iron or steel sheets or plates, bars, tubes, wire, and articles fabricated from iron or steel by operations involving pressing, stamping, rolling, grinding or machining.

A principal object of this invention is the inhibition or prevention of rusting of ferrous metal surfaces by the application thereto of a film of oil containing a small quantity of a synthetic ester of an organic acid, preferably a relatively non-volatile synthetic ester of a carboxylic acid having from about 8 to about 25 carbon atoms per molecule, and boiling above about 200° C.

The oils to be employed in accordance with this invention are preferably hydrocarbon oils having a Saybolt Universal viscosity at 100° F. of at least 60 seconds, and substantially free of constituents tending to stain, corrode or react with ferrous metal surfaces. Hydrocarbon oils derived from paraffin base or naphthene base petroleum, or oils produced by solvent extraction, hydrogenation or other means may be suitably employed. In general the oil component of the rust-preventing composition comprises about 90% or more of the composition.

The synthetic esters to be employed in conjunction with the hydrocarbon oil are preferably those derived by the reaction of aliphatic or aromatic alcohols or phenols with carboxylic acids, preferably saturated carboxylic acids having from about 8 to about 25 carbon atoms per molecule. Among the alcohols may be mentioned methyl alcohol, ethyl alcohol, propyl alcohol, isopropyl alcohol, the butyl alcohols, the amyl and hexyl alcohols, cetyl alcohol, the glycols, glycerol, phenol, cresol, naphthol, benzyl alcohol and the like. The organic acids may be exemplified by caprylic acid, capric acid, undecylic acid, lauric acid, myristic acid, palmitic acid, margaric acid, stearic acid, arachidic acid, cerotic acid, melissic acid, the naphthenic acids, benzoic acid, phthalic acid and the like. Quantities of the esters of the order of 1%, 2%, 5%, and 10% or more may be added to the hydrocarbon oil and the admixture or solution applied to rustable metal surfaces by dipping, spraying, painting or other means.

It has been found that oil-synthetic ester compositions employed in accordance with the present invention, when applied to ferrous metal surfaces, provide a fluid film which is tenaciously

held by the metal surface, probably by adsorption, and which is resistant to the penetration of moisture. Such films are non-drying and readily removable by wiping, washing with organic solvents, soap solutions or other detergents. The oil-synthetic ester compositions utilized in accordance with this invention do not have the disadvantages inherent in the use of natural oils, fats, fatty oils and mixtures thereof with hydrocarbon oil, which have been employed heretofore as rust-proofing agents. Many of the natural fatty oils are glycerides of unsaturated fatty acids, and when applied to metal surfaces in the undiluted state or admixed with hydrocarbon oil, form sticky or tacky films due to the oxidation and/or polymerization of the unsaturated constituents. These tacky films are difficult to remove, since the oxidized constituents are relatively insoluble in organic solvents and not readily removed by water or detergent solutions. Furthermore, many of the fatty oils contain varying amounts of free fatty acids which tend to corrode or stain the metal with which they come in contact. The fatty oils also tend to become rancid, particularly when exposed in relatively thin films to the action of air. However, the synthetic esters employed in conjunction with hydrocarbon oil in accordance with this invention do not form sticky or gummy deposits upon the metal surfaces, do not oxidize nor polymerize, nor become acidic nor rancid, and are readily removed from metal surfaces.

The following examples will serve to further illustrate my invention. Test pieces of polished, cold rolled steel were coated with the rust-inhibiting compositions and exposed to the atmosphere (temperature 77° F.; humidity 100%) for a period of one week. The viscosity of the mineral oil component is given in seconds Saybolt Universal at 100° F.

| Rust-inhibiting composition                | Appearance of steel test piece |
|--------------------------------------------|--------------------------------|
| 62 vols. paraffin oil                      | Very bad rusting.              |
| 62 vols. paraffin oil + 2% butyl stearate  | Slight rusting.                |
| 100 vols. paraffin oil                     | Very bad rusting.              |
| 100 vols. paraffin + 2% butyl naphthenate  | Slight rusting.                |
| 250 vols. paraffin oil                     | Very bad rusting.              |
| 250 vols. paraffin oil + 5% butyl stearate | Very slight rusting.           |

From the above examples it will be seen that the hydrocarbon oil, per se, was ineffective as a rust-inhibitor, whereas the hydrocarbon oil-synthetic ester compositions showed a marked inhibiting action and prevented rusting to a satis-

factory extent. The rust inhibiting method of the present invention is particularly adapted for the protection of iron or steel products which may be placed in storage under conditions normally conducive to rusting.

For brevity, herein and in the appended claim, the term "viscous hydrocarbon oil" is to be understood to comprehend oils having a Saybolt Universal viscosity at 100° F. of 60 seconds or higher.

What I claim is:

A method of inhibiting rusting of a ferrous

metal surface which normally is subjected to oxidation and rusting conditions which comprises applying to said metal surface a substantially non-sticky and non-gummy film of viscous hydrocarbon oil substantially free from constituents tending to stain, corrode, or react with the ferrous metal surface, containing of the order of 10% of a relatively non-volatile synthetic ester from the group consisting of alkyl stearates and naphthenates.

WILLIAM K. GRIESINGER.

5

10